

July 11, 1933.

C. J. COBERLY

1,917,497

METHOD OF DRAWING TEMPER IN CUTTING SLOTS

Filed April 15, 1930

*Fig. 1.*



*Fig. 3.*



*Fig. 2.*



*Fig. 4.*



*Fig. 5.*



*Fig. 6.*



INVENTOR:  
Clarence J. Coberly.  
BY

*Ed. W. Martin*

ATTORNEY.

## UNITED STATES PATENT OFFICE

CLARENCE J. COBERLY, OF LOS ANGELES, CALIFORNIA, ASSIGNEE TO KOBE, INC., OF HUNTINGTON PARK, CALIFORNIA, A CORPORATION OF CALIFORNIA

## METHOD OF DRAWING TEMPER IN CUTTING SLOTS

Application filed April 15, 1930. Serial No. 444,495.

My invention relates to the art of cutting slots in metal by use of a gas jet and relates particularly to the cutting of slots in metal walls whereby to form screen, strainers or filters therefrom.

My invention is of special utility in the cutting of slots in pipes by use of oxygen jets, these pipes being then suitable for use as screen or strainers in wells.

The present practice of cutting slots in pipe includes first the drilling of a small hole at which to start a slot, preheating the metal surrounding the hole to such temperature that combustion of the metal will take place in the presence of an oxygen jet, directing a cutting jet of oxygen through the hole and moving the oxygen jet so as to cut a slot in the pipe. During the slotting operation and subsequent thereto cold air is drawn through the slot for the purpose of rapidly cooling the heated walls of the slot in order to harden such walls and thus equip the walls for greater resistance to abrasion by materials carried in the fluids, which are to subsequently pass through the slot.

It is found that this process, which is followed through in the cutting of a slot, produces slot walls which are harder at the finishing end of the slot than at the starting end thereof, which is an undesirable condition especially where alloy steels are employed in the pipes.

My invention embraces a new and simple method whereby an isothermal condition will be maintained in the metal surrounding the slot and will operate to equalize the temper of the slot walls throughout their lengths. The conditions existing in the present practice of cutting slots by use of a gas jet and a clear understanding of the improvement accomplished therein by the use of my present invention will be made evident in the following part of the specification.

Referring to the drawing, which is for illustrative purposes only,—

Fig. 1 is a vertical partly sectioned view showing a metal wall, in which a hole has been drilled at which to start a slot and showing a cutting torch in position for preheating

preliminary to cutting a slot by use of an oxygen jet.

Fig. 2 is a fragmentary plan view corresponding to Fig. 1 showing the portion of the metal wall in which a slot is to be cut. 55

Fig. 3 is a view similar to Fig. 1 showing the position of the cutting torch at the completion of the slotting operation.

Fig. 4 is a plan view corresponding to Fig. 3 showing on the surface of the metal wall an isothermal line indicating the thermal condition of the metal surrounding the slot.

Fig. 5 is a view similar to Fig. 1 showing the manner in which the cutting torch may be employed to correct the unsatisfactory thermal condition of the metal surrounding the slot at the completion of the cutting of the slots by the oxygen jet. 65

Fig. 6 is a plan view corresponding to Fig. 5, showing on the surface of the metal wall 70 the isothermal line existing at the completion of my present slot cutting method.

In Figs. 1 and 2, I show a metal plate 11, such as the wall of a pipe, in which slots are to be cut. To provide a starting point for the cutting of the slot by use of an oxygen jet, a small hole 12 is drilled through the plate 11. A cutting torch is so placed that the tip 13 thereof will align with the hole 12 and the metal surrounding the hole 12 is preheated by 75 the heating flames 14 of the cutting torch tip 13 to bring the metal adjacent the hole 12 into condition for combustion in the presence of the oxygen jet issued from the cutting torch tip 13. The cutting torch tip 13 is held stationary in the position which is indicated in Fig. 1 until completion of the preheating operation, then as indicated by dotted lines 15 in Fig. 3, an oxygen jet is directed through the hole 12 from the cutting torch tip 13 and the tip 13 is moved in rightward direction 80 whereby to cut a slot 16 in the plate 11. In customary slotting practice when the tip 13 reaches the end of its cut, such as the position indicated at 17 in Fig. 3, the oxygen jet 85 is cut off and the tip 13 is removed to a new position, or the heating flames are discontinued, the result being that as soon as the slot is cut by the oxygen jet no further heat is delivered to the metal surrounding or adj- 90

100

cent to the rear end of the slot. It is therefore characteristic of the ordinary method of slot cutting that an unbalanced or unequalized thermal condition exists in the metal of the plate 11 immediately surrounding the slot 16.

Referring to Fig. 2, the play of the heating flames 14 on the metal surrounding the hole 12 preliminary to cutting a slot in the plate 11 results in heat flowing upwardly in the metal surrounding the hole, as indicated by the circular isothermal line 18. During actual cutting by the oxygen jet, the heating flames 14 are moving across the plate 12 so that the amount of heat delivered into or absorbed by the metal adjacent the slot 16 is reduced, the result being that the combined heat of the heating flames and the heat generated by the slot cutting operation produces an isothermal line 20 around the completed slot 16, as shown in Fig. 4, indicating an unbalanced thermal condition in the metal adjacent opposite ends of the slot 16. In order to harden the walls 21 of the slot 16, air is drawn through the slot 16 as indicated by arrows 22 in Fig. 3 during and subsequent to the cutting of the slot. The action of the oxygen jet 15 in causing the cutting of metal from the plate 11 to form the slot 16 produces a very high temperature in the surface portions of the slot walls 21 so that these slot walls are readily hardened in the presence of the air blast which is drawn through the slot, as indicated by arrows 22, especially where the plate 11 is made of alloy steel having pronounced hardening characteristics.

As diagrammatically indicated by the area 23 outlined by the isothermal line 20 of Fig. 4, more heat is stored or contained in the metal adjacent the front end 24 of the slot 16 than in the metal adjacent the rear end 25 of the slot. The heat present in the metal walls adjacent to the slot acts to temper the hardened surface portions of the slot walls 21 so as to relieve possible brittleness thereof, or to reduce their hardness, this tempering action being in proportion to the amount of heat stored in the metal adjacent the slot 16 and is therefore proportionate to the width of the area 23, which graphically represents the heat stored in the consecutive portions of metal lying along the slot 16. The difference between the thermal condition of the metal adjacent to the front end 24 of the slot 16 and the metal adjacent the rear end of the slot 16 results in the slot walls 21 being of a lesser hardness at the front end 24 of the slot than at the rear end 25 thereof, and should a slot cut in the manner previously described be of proper slot wall hardness at the front end 24 of the slot 16, the rear end of the slot will be too hard and possible brittle so as to offer poor resistance to abrasion by sand. Conversely to this, should the slot walls 21 be of proper hardness at the rear end of the slot,

the slot walls at the front end of the slot would be of insufficient hardness.

Figs. 1 to 4 show the first part of my invention of a new slotting method and also the slotting method as previously practiced, indicating together therewith the disadvantages encountered in the previous method of slotting metal plates.

My new method is practiced substantially as follows:

A hole 12 is drilled in the metal plate 11 and the flames 14 of the cutting torch tip 13 are directed against the metal surrounding the hole 12 for a sufficient length of time to accomplish the desired preheating thereof. The oxygen valve of the cutting equipment is then opened and a cutting jet 15 is directed through the hole 12 whereupon the tip 13 is moved from its dotted line position in Fig. 3 to its full line position therein, cutting the slot 16 as the result of such movement. At the end of the slot 16 the oxygen jet 15 is discontinued, but, as indicated in Fig. 5, the torch tip 13 is maintained in position at the end of the slot 16 and the heating flames 14 thereof are caused to play on the metal adjacent the rear end of the slot for a period of time substantially equal to the time necessary to preheat the metal surrounding the hole 12 preliminary to turning on the oxygen jet of the torch, the result of this being that an amount of heat is absorbed by the metal adjacent the rear end 25 of the slot 16 to produce a thermal condition surrounding the slot 16, as indicated by the isothermal line 30 of Fig. 6. The isothermal line 30 outlines an area 31 which graphically indicates the thermal condition existing in the metal adjacent the consecutive portions of the slot 16. This area 31 is of equal width at its ends, and of but slightly reduced width at its center. Due to the balanced heat condition in the metal along and at the ends of the slot 16, it may be said that by the practice of my new method, an isothermal condition is maintained or established in the metal of the plate 11 surrounding the slot 16, and by tests of the surface hardness of the walls of a slot cut by my new method it is shown that as the result of such isothermal condition a substantially constant hardness is maintained throughout the entire length of the slot.

The practice of my new invention therefore accomplishes the production of slot walls better adapted for use in oil well screen or for strainers, than the slot walls produced by the previous method of cutting slots by the use of oxygen jets. No strains or unequalized stresses are produced in the metal adjacent opposite ends of the slot and accordingly greatest strength and durability is maintained in the metal wall in which the slots are formed.

I claim as my invention:

1. A method of the character described for

equalizing thermal conditions in metal surrounding a gas-cut slot, consisting of applying an excess of heat to the metal adjacent to the rear end of the slot sufficient in quantity 5 to produce an isothermal condition in the metal surrounding the slot.

2. A method of the character described for equalizing thermal conditions in metal surrounding a gas-cut slot, consisting of applying 10 heat to the metal adjacent to the slot after termination of the cutting operation.

3. A method of the character described for equalizing thermal conditions in metal surrounding a gas-cut slot, consisting of applying 15 a flame to the metal adjacent to the rear end of the slot for a sufficient time to produce a substantially isothermal condition in the metal surrounding the entire slot.

4. A method of the character described for 20 equalizing thermal conditions in metal surrounding a gas-cut slot, consisting of applying a flame to the metal adjacent to the rear end of the slot for a sufficient time after completion of the slot to produce an isothermal 25 condition in the metal surrounding the slot.

5. A method of the character described for equalizing thermal conditions in metal surrounding a gas-cut slot, consisting of applying heat at a point along said slot and spaced 30 from the front end of the slot after termination of the cutting operation to produce an isothermal condition in the metal surrounding the slot.

6. A method of cutting slots in metal in a 35 manner to produce an isothermal condition in the metal immediately surrounding said slot, comprising: directing a preheating flame to preheat said metal at the starting point of the slot to be made; creating a gas 40 jet to cut said metal at said starting point; moving said jet so as to cut a slot in said metal; and directing a flame against the metal adjacent to the position of the rear end of said slot for a period of time sufficient to 45 produce a substantially isothermal condition in the metal surrounding said slot.

7. A method of the character described for 50 equalizing thermal conditions in metal surrounding a gas-cut slot, consisting of applying heat to the rearward part of the area of metal surrounding the position of said slot

in addition to the ordinary heat of the slot-cutting operation and sufficient in quantity to produce a substantially isothermal condition in the metal surrounding the slot.

8. A method of the character described for 70 equalizing thermal conditions in metal surrounding a gas-cut slot, consisting of applying heat in addition to the ordinary heat of the slot-cutting operation to the area of metal adjacent a part of said slot following the 75 front end of said slot, so distributed and proportioned in quantity as to produce a substantially isothermal condition in the metal surrounding the slot.

9. A method of the character described, 80 consisting of: preliminarily heating an area of a piece of metal to raise the temperature to permit a burning of the metal; directing a jet of cutting gas through said metal and moving same therealong to form a slot; and, 85 after said slot-forming operation, heating the metal at the finishing end of said slot to substantially the same amount as the metal at the starting end of said slot was heated.

10. A method of cutting a slot in metal by 90 use of a gas-operated cutting torch, said method including: applying heating jets of said torch to said metal to preheat same; directing a cutting jet of said torch through said metal; moving said torch relative to said 95 metal; discontinuing the directing of said cutting jet through said metal; and applying said heating jets to said metal at the finishing end of the slot formed by said cutting jet, for substantially the same duration 100 as said heating jets were applied at the starting end of said slot.

11. A method of the character described, 105 consisting of: preliminarily heating an area of a piece of metal to raise the temperature to permit a burning of the metal; directing a jet of cutting gas through said metal and moving same therealong to form a slot; and, 110 after said slot-forming operation, heating the metal at the finishing end of said slot to produce a substantially isothermal condition in the walls of said slot.

In testimony whereof, I have hereunto set my hand at Los Angeles, California, this 115

10th day of April, 1930.

CLARENCE J. COBERLY.